

## UNITED STATES PATENT OFFICE.

FAY C(LUFF) BROWN, OF IOWA CITY, IOWA.

## SELENIUM CRYSTALS AND METHOD OF PREPARING THE SAME.

No Drawing.

Application filed March 7, 1916. Serial No. 82,782.

*To all whom it may concern:*

Be it known that I, FAY C. BROWN, a citizen of the United States, residing at Iowa City, in the county of Johnson and State of Iowa, have invented new and useful Selenium Crystals and Methods of Preparing the Same, of which the following is a specification.

This invention has reference to selenium crystals and its object is to produce light sensitive selenium crystals of greatly increased sensitiveness.

It has long been known that selenium in some of its forms is less resistant to the passage of an electric current when under the influence of light than when in the dark, that is, protected from the action of light. Advantage has been taken of this property of selenium for various purposes and the devices for utilizing the selenium in such manner have been customarily known as selenium cells, but such term is somewhat of a misnomer, wherefore the term selenium bridge is used throughout this specification, because the selenium is utilized to bridge a gap in the electric circuit, whereby the variable resistance represented by the selenium may be utilized.

Prior to the present invention crystallized selenium has been produced, but the crystals have been of comparatively small size. For this reason there can be no control of the arrangement of the crystals which because of their extremely small size are present in great multitudes in the ordinary selenium bridge. Such crystals have their axes pointing in all directions.

By the production of crystals of selenium of large size, that is, readily visible individually to the unaided eye and easy to handle, it is quite possible to produce a selenium bridge of suitable capacity from a single crystal, and the capacity may be increased by the employment of two or three or more crystals, for the crystals are of such large size as to be readily oriented. It has been found that a single hexagonal crystal shows a greater sensibility to light when the illumination impinges on the end of the crystal and travels in the direction of the principal axis of the crystal.

Moreover, it has been found that such crystals when subjected to pressure exhibit a many fold increase in sensitiveness to the action of light, so that a selenium crystal so arranged that the light strikes it in the di-

rection of its principal axis and under compression to a considerable degree, is increased in light sensitiveness, say, a thousand times over the sensitiveness of selenium bridges as heretofore constructed.

The selenium bridge of the present invention, therefore may comprise one or more crystals of selenium with means for subjecting such crystal or crystals to pressure and at the same time having the crystals so presented that the light rays strike them in the direction of their principal axes.

The invention will be best understood from a consideration of the following detailed description.

In using selenium crystals, made after the manner herein described, for selenium bridges whose resistance varies in accordance with the amount of light impinging thereon, certain precautions should be observed, if the best results are to be secured. The selenium crystal is placed in the circuit between the electrodes of any suitable material, for example, those hereinafter mentioned. Increased sensitivity results from applying pressure to the crystal and in the case of hexagonal crystals it is advantageous to apply the light ray in the direction of the principal axis of the crystal. The crystal may be shielded from extraneous light in any suitable manner and a window or opening may be provided through which the varying light ray may impinge upon the crystal. For a more detailed description of the possible uses to which such crystals may be put and of the precautions to be observed in using them reference may be made to the specification of my United States Patent 1,219,432, patented March 20, 1917.

Selenium exists in the amorphous or non-conducting form, in the red crystalline form, also non-conducting, and in a crystalline metallic state with the crystals of monoclinic or hexagonal shape very sensitive to light and with properties peculiar to the various axes of the crystals and also due to the manner of operation of the crystals.

In the light sensitive crystalline form utilized in the present invention, isolated crystals ranging from 4 mm. to 9 mm. long, and even longer, have been produced by sublimation of the selenium vapor either in a high vacuum or at atmospheric pressure. When the selenium is sublimed in a high vacuum it is first freed from all occluded gases, wherefore the sealed receptacle con-

tains nothing but selenium which becomes vaporized by the heat employed and from which vapor the crystals are deposited. The crystals are of the monoclinic form when the 5 temperature is about 171° C. Hexagonal crystals of a maximum sensibility to light are obtained when the vapor is sublimed at a temperature of about 183° C.

A high sensitiveness has been obtained 10 when occluded gases have been driven off from the selenium by repeated boiling and condensing in a high vacuum. For some purposes it is advantageous to have argon, neon, helium and other gases mixed with the 15 vapor of selenium either separately or in combination, and, again, it is advantageous to form the crystals in an atmosphere of selenium vapor only and afterward allow them to absorb any one gas or a mixture of 20 the gases at temperatures below the temperature of formation.

While the temperatures named have been found to produce most excellent results, it is to be understood that the invention 25 is not in any manner limited to any precise temperatures.

One method of producing the herein described sensitive selenium crystals of high sensitivity will be described in detail. Vitreous 30 selenium which is to be transformed into crystals is placed in one end of a glass tube of about 35 mm. inside diameter and of about 30 to 60 cm. length. This tube is placed in a cylindrical electrical oven of 35 about 30 cm. length closed at one end. A suitable current is used to heat the selenium to a sufficiently high temperature to cause it to vaporize. The glass tube may be highly 40 evacuated, filled with some of the various gases hereinbefore mentioned, or filled with ordinary air at atmospheric or lower pressures. In general the use of air is not recommended, but its elimination is not essential for all purposes. Where the glass tube 45 projects from the oven will be a region of high temperature gradient. The apparatus should be set up and maintained quietly for a long period which may vary in accordance with circumstances from a minimum of one 50 day to a maximum of one week or more. Along the part of the tube where the temperature gradient is the greatest will be found numerous crystals. In general the largest crystals will be formed at the point of highest 55 temperature at which the selenium will sublime. In various parts of the region in which crystallization takes place there will occur various forms of selenium crystals. It is not possible to determine in advance or 60 predict with certainty the form which the crystals will take in any particular instance or the relative quantities or sizes of the various types, or the size of individual crystals. It will happen, however, that certain 65 crystals will be relatively large, that is

of a length of 4 mm. and upward. The smaller crystals and the selenium which is deposited in non-crystalline form may be resublimed either with or without the addition of other selenium. The resublimation 70 may be performed under the same or different conditions as the first sublimation as may be desired.

For further and more detailed information reference may be made to an article by 75 me on the "Crystal forms of metallic selenium and some of their physical properties," published in Physical Review, N. S., vol. 4, No. 2, August 1914.

A single crystal of a substance is more 80 likely to be pure and of the same crystalline structure throughout than is the case with a heterogeneous mass of material, wherefore such crystal has the advantage 85 of a uniform molecular structure throughout, that is, a uniform and regular spacing of the molecules. Such uniformity of structure contributes to the stability of the crystal and of the selenium bridge in which the 90 crystal is included.

Large crystals are advantageous in that 95 because of the parallel plane faces of the crystal it is possible to apply pressure on the electrodes after the crystals are formed. The pressure on a single crystal or an assemblage of single crystals is more likely 100 to produce a uniform stress in the crystal or crystals than is the case where pressure is applied to a mass-aggregate of sub-microscopic crystals.

Large crystals permit pressure to be applied with so simple a device as a screw, and also permit the control of the axis along which the crystal may be illuminated. Not only is the sensibility different, dependent upon the orientation of the axis to 105 be illuminated, but this orientation determines which region of the spectrum will produce the maximum change of conductivity.

Experience has shown great stability of 110 the new crystals of selenium over selenium as hertofores used in selenium bridges. A selenium crystal as produced and employed in accordance with the present invention 115 has been exposed to most intense light for twenty-four hours a day for thirty-five days without showing deterioration. Such a crystal mounted for a year has now the same sensibility as when first mounted.

The electrodes may be made of a material 120 that does not attack the selenium chemically. For instance, platinum answers the purpose excellently, and in all probability tungsten, or carbon in some one of its 125 forms, or other substances may be employed.

A bridge may comprise a group of much 130 smaller crystals than those of the particular sizes mentioned hereinbefore, and especially crystals which may be deposited from

- selenium vapor. It is not imperative that the light affecting the bridge shall reach the crystal or crystals in the direction of the principal axis thereof. For instance, 5 the crystals may be illuminated through one of the electrodes which might be accomplished by employing an electrode consisting of a glass or quartz plate provided with a thin coating of platinum.
- 10 Selenium crystals made in accordance with the methods herein set forth may be used for any desired purpose. Certain uses are described in my patent referred to above.
- 15 What is claimed is:—
1. The method of preparing selenium for use in selenium bridges, which consists in freeing selenium from occluded gases, then vaporizing the selenium by heat in a high 20 vacuum, and causing the deposition of crystals from the selenium vapor so produced.
  2. The method of preparing selenium crystals for use in selenium bridges, which consists in freeing the selenium from oc- 25 cluded gases, then heating the selenium in a high vacuum to produce selenium vapor, and causing the deposition of crystals of selenium from such selenium vapor, and finally causing the crystals so formed to 30 absorb one or more gases.
  3. The method of making selenium crys- tals by sublimation comprising vaporizing the selenium in a vacuum.
  4. The method of making selenium crys- 35 tals from selenium by sublimation comprising eliminating occluded gases from the selenium and vaporizing the selenium in a vacuum.
  5. The method of making selenium crys- tals from selenium which comprises vapor- 40 izing selenium and precipitating the vapor under conditions which prevent the occlusion of undesired gas in the resulting crys- tals.
  6. The method of making selenium crys- tals from selenium comprising vaporizing the selenium and precipitating the vapor at a temperature of approximately 180° C. 45
  7. A selenium crystal having occluded therein inert gas substantially exclusively. 50
  8. A selenium crystal having occluded therein gas principally of the helium group.
  9. The method of making selenium crys- tals from selenium by sublimation, comprising vaporizing the selenium in a closed 55 vessel at substantially less than atmospheric pressure, and maintaining the vessel under uniform conditions of temperature and pressure for a long period of time to cause the deposition of the selenium vapor in the form of the desired crystals.
  10. The method of preparing selenium crystals comprising repeatedly vaporizing and condensing selenium in an evacuated 60 vessel. 65
  11. The method of producing sensitive selenium crystals, comprising repeated sublimation of selenium in a vessel from which the larger part of the atmosphere has been removed. 70
- In testimony that I claim the foregoing as my own, I have hereto affixed my signature in the presence of two witnesses.
- FAY C(LUFF) BROWN.
- Witnesses:
- HOMER L. DODGE,  
L. E. DODGE.